

# United States Patent

## Humphries

[15] 3,681,911  
[45] Aug. 8, 1972

[54] **SEALED WIRE ROPE AND STRAND  
AND METHOD OF MAKING SAME**

[72] Inventor: **Darral V. Humphries, Allentown,  
Pa.**

[73] Assignee: **Bethlehem Steel Corporation**

[22] Filed: **March 30, 1971**

[21] Appl. No.: **112,211**

**Related U.S. Application Data**

[63] Continuation-in-part of Ser. No. 850,148, Aug.  
14, 1969, abandoned.

[52] U.S. Cl. .... **57/149, 57/153, 57/162,  
57/164, 161/175, 117/128**

[51] Int. Cl. .... **D07b 1/16, D02g 3/36**

[58] Field of Search .... **57/140 R, 140 C, 149, 153,  
57/162, 164; 161/172, 175; 117/127, 128,  
128.4, 128.7, 132, 133**

[56]

**References Cited**

**UNITED STATES PATENTS**

|           |        |                      |             |
|-----------|--------|----------------------|-------------|
| 3,370,045 | 2/1968 | Sadle .....          | 117/128.4 X |
| 3,463,652 | 8/1969 | Whitesel et al. .... | 57/149 X    |
| 3,507,741 | 4/1970 | Aleixo .....         | 57/153 X    |
| 3,589,121 | 6/1971 | Mulvey .....         | 57/149 X    |

**FOREIGN PATENTS OR APPLICATIONS**

|         |        |                    |        |
|---------|--------|--------------------|--------|
| 789,163 | 1/1958 | Great Britain..... | 57/153 |
| 954,514 | 4/1964 | Great Britain..... | 57/149 |

*Primary Examiner*—Donald E. Watkins

*Attorney*—Joseph J. O'Keefe

[57] **ABSTRACT**

A wire rope or strand is provided with a plastic foam type internal sealant to cushion the wires and strands and provide corrosion protection.

**16 Claims, 12 Drawing Figures**



PATENTED AUG 8 1972

3,681,911

SHEET 1 OF 2



INVENTOR  
*Darral V. Humphries*

PATENTED AUG 8 1972

3,681,911

SHEET 2 OF 2



INVENTOR  
Darral V. Humphries

**SEALED WIRE ROPE AND STRAND AND METHOD  
OF MAKING SAME**

**CROSS-REFERENCES TO RELATED  
APPLICATIONS**

This application is a continuation-in-part of U. S. application Ser. No. 850,148 filed Aug. 14, 1969, now abandoned.

**BACKGROUND OF THE INVENTION**

This invention relates to the sealing of wire rope and strand for protection against corrosive environments.

Steel wires and strands are subject to internal corrosion of wires due to the entrapment of water within the structure of the strand between the individual wires.

Various expedients have been used to bar the entrance of the water including the provision of heavy lubricants, external plastic coating and encapsulation of the individual wires, strands, or even an entire wire rope, in solid plastic sheaths. Lubricants are soon lost from an otherwise unprotected rope or strand. External coatings and sheaths are subject to wear, and upon rupture of the sheath at any point will admit moisture to the entire strand or rope. Solid encapsulation of a rope or strand on the other hand not only makes the structure too stiff and inflexible for many uses but is also difficult to attain.

Encapsulation of individual wires prior to fabrication also results in considerable stiffening of a rope subsequently fabricated from the wires and the wire density in the rope is undesirably reduced by the additional thickness of the plastic. In addition the corrosion protection afforded to the wires by the plastic polymer coating is lost if the coating is damaged during rope or strand manufacture, a rather common occurrence.

Various expedients have been tried to alleviate the foregoing difficulties but none has heretofore been completely successful. The present invention prevents the entrance into and migration of moisture in liquid or vapor form through a wire rope or strand while avoiding the foregoing disadvantages of the prior art.

**SUMMARY OF THE INVENTION**

In the practice of the present invention the individual wires or strands of a strand or rope are initially coated with a heat foamable plastic composition and subsequently after fabrication of the wires or strand into a wire rope the body of the rope is heated while confined within a conforming mold to expand the plastic into a substantially closed cell plastic foam. The plastic foam is light and flexible, prevents the entrance and migration of moisture into and through the internal portions of the rope, provides a cushion for the strands and does not significantly decrease wire density in the strand or rope. The plastic foam also acts as a vibration damper when the rope is subjected to fluctuating loads in service. Since the foaming of the plastic is not carried out until the fabrication of the rope or strand has been completed the foam plastic coating on the wires is self-healing and any damage to the plastic during fabrication of the strand or rope is healed over during the foaming step. A plastic foam coating, furthermore, is economical due to the low average density of the plastic filling between the wires and strands of the rope. A dense outer layer of denser wear resistant plastic encapsulates the foam filled rope or strand.

**BRIEF DESCRIPTION OF THE DRAWINGS**

FIG. 1 schematically shows a fabrication line for parallel wire strand incorporating a plastic foam sealing step.

FIG. 2 is a cross-sectional elevation of a portion of FIG. 1 showing a plastic coating bath.

FIG. 3 is an enlarged cross-sectional view along line 3-3 of FIG. 1.

FIG. 4 is an enlarged cross-sectional view along line 4-4 of FIG. 1.

FIG. 5 is an enlarged cross-sectional view along line 5-5 of FIG. 1.

FIG. 6 shows a section of wire rope undergoing a batch type foaming operation.

FIG. 7 is an enlarged cross-section along 7-7 of FIG. 6.

FIG. 8 is an enlarged cross-section along 8-8 of FIG. 6.

FIG. 9a is an enlarged cross-section along 9-9 of FIG. 6.

FIG. 9b is a further enlarged half section of FIG. 9a.

FIG. 10 is a schematic representation of an apparatus for continuously foaming plastic in wire rope.

FIG. 11 is a cross-sectional view along 11-11 of FIG. 10.

**DESCRIPTION OF THE PREFERRED  
EMBODIMENTS**

In FIG. 1 is shown a parallel wire strand fabrication line adapted for the production of foam filled parallel wire strand.

Two groups of reels 11 and 13 rotatable in opposite directions are arranged to provide wires 15 and 17 for fabrication into a parallel wire strand. Wires 15 from reels 11 are guided by small guide plates 19 to plastic coating chamber 23 where the wires are coated with a foamable plastic composition. Wires 17 from reels 13

are in like manner guided to coating chamber 23 by guide plates 25. The wires 15 and 17 may be coated in chamber 23 in any convenient manner, but as illustrated the wires are deflected by guide rollers 27 within chamber 23 into and below the surface of a bath of a foamable plastic composition 28. The bath is composed of a suspension or solution of foamable plastic material in a solvent. The wires 15 and 17 then pass through wiping dies 29 located in the side of coating chamber 23 and pass to drying chamber 31 where the foamy composition is firmly dried upon the individual wires by exposure to a low heat to evaporate the solvent from the plastic composition and form a coating 30 of foamy plastic upon the individual wires. As the wires pass from coating chamber 23 to drying chamber 31 they may be exposed to an air blast from compressed air nozzle 33.

From drying chamber 31 the wires 15 and 17 with coatings 30 pass through a series of converging lay plates 35, 37 and 39 which direct the two groups of wires into a first die 41. Die 41 may be a roller type die to reduce friction. Lay plates 35, 37 and 39 will desirably have anti-friction surfaces within their guide holes such as polytetrafluoroethylene inserts or even roller type bearing surfaces in order not to scrape the solidified foamy plastic coating 30 from the wires.

The wires 15 and 17 pass from die 41 to an identical die 43. The wires are formed in these two dies into a

parallel wire strand 45. Preferably dies 41 and 43 will have a hexagonal cross-section so as to form a hexagonal parallel wire strand as disclosed in U. S. application Ser. No. 575,038, filed Aug. 26, 1966, now U. S. Pat. No. 3,526,570, issued Sept. 1, 1970, by Durkee et al. for Parallel Wire Strand. The hexagonal shape of the strand 45 aids in obtaining an effective grip upon all the wires of the strand to pull them evenly through the dies and prevent rotation of the wires as taught in the referred to application. It will be understood, however, that the cross-sectional shape of the strand may take other configurations besides hexagonal if the exact disposition of the wires in the strand is not critical in the parallel wire strand being fabricated.

In the dies 41 and 43 the wires of the strand are subjected to considerable transverse force which deforms the foamable plastic coating 30 on the wires at the contact line between the wires so that the resultant strand has a high wire density with a minimum separation between the bodies of the wires.

From die 43 strand 45 passes to mold 47 which may be formed from some dielectric substance such as hard rubber, plastic or other similar composition. Preferably mold 47 is water-cooled through inlet pipe 49 and hose 49a and outlet pipe 51 and hose 51a. Within the mold the cooling water flows through cooling pipes 50 shown in FIG. 4. Mold 47 has an internal cross-section identical in size and shape with the shape and outside dimensions of the parallel wire strand 45.

Induction heating rings 53 surround the initial sections of mold 47 to heat the wires of the strand therein to a temperature sufficient to melt the plastic coating 30 on the wires and cause the foaming agent therein to expand the plastic into a plastic foam 55. The strand 45 then passes through the portion 57 of the mold 47 through which the cooling water initially passes and about which no induction heating coils are disposed. The strand 45 and foamed plastic 55 are cooled in this section of the mold to set the plastic.

The strand 45 then passes from mold 47 to dies 59 and 61, which are preferably roller type dies, and is wrapped between the dies at spaced intervals along the strand as it passes between the two dies with a plastic tape or other securing means to maintain the shape of the strand. The wrapping may be applied manually or by means of any suitable automatic wrapping machine.

After the wrapped strand passes through die 61 it passes to any suitable catapuller device 63 which serves to pull wires 15 and 17 and the strand 45 from the respective reels and through the previous apparatus. From catapuller 63 the strand passes through a traverse device 65 and is reeled onto a large diameter reel 67.

As the strand passes through mold 47 its component internal wires are heated by currents induced in the wires by the conduction coils and the plastic composition on the wires foams as shown in FIG. 4 and is then cooled into a permanent plastic foam seal 69 between the internal wires of the strand as shown in FIG. 5. The cooled close-fitting internal surface of the mold 47 prevents the plastic on the wires at the surface of the strand from foaming to any significant degree, forms a thin layer 5b of fairly dense solidified plastic near the surface of the strand as best seen in FIG. 5, and forces the foamed plastic deep into the strand between the wires.

The plastic foam 55 completely fills the interstices between the wires effectively sealing the strand against the entrance into or migration through the strand of any corrosive agents. The plastic foam 55 is flexible and has little bulk so that it neither interferes with the flexibility of the strand as in reeling upon reel 67 nor decreases the wire density within the strand significantly. The term "wire density" as used in this application refers to the amount of space in the strand physically occupied by the component wires.

The plastic foam can be of any suitable composition such as a vinyl plastic having an organic nitrogen compound such as azodicarbonamide as a foaming agent. This plastic when heated above the decomposition temperature of the organic nitrogen compound decomposes into nitrogen and carbon dioxide and expands the plastic into a foam. Another suitable composition would be a foamable polyurethane consisting of a thermosetting elastomer filled with expandable plastic beads. When exposed to heat the plastic of the beads softens and an entrapped gas therein expands the plastic into a foam. The polyurethane elastomer matrix provides cross linking. Any other plastic composition which is flexible, tough and adherent to metal may be used with a foaming agent to coat the strand.

In FIG. 6 is shown a section of fabricated wire rope 71. The individual wires 73 of the rope 71 have before fabrication into strands 75 been coated with a plastic foamable composition 76 in some suitable manner such as, for instance, shown in FIG. 1. The strands 75 are then stranded into the main rope 71 as is well known in the art.

Any section of the rope 71 which it is desired to impregnate with plastic foam may then be placed within mold 77 which is formed from a dielectric material. The internal section of the mold has a spiral configuration conforming to the spiral arrangement of the strands 75 of the rope 71. The mold 77 is formed in two halves 79 and 81 so it may be conveniently placed around the strand and is provided with a spiral internal configuration to conform with the helical lay of the strands of the rope. It may be convenient in some instances to form the mold from more than two major sections in order to facilitate assembly over the rope. If desired the mold may be water cooled, particularly if it is to be used repetitively. If the mold is formed from hard molded rubber it will conform quite well to the surface of the wire rope preventing foaming of the plastic on the external surface of the rope and forcing the major portion of foaming composition into the interior of the strands and the interior of the rope between the strands.

In order to foam the plastic an induction coil 83 is passed over the mold sections 79 and 81 after they are placed over the wire rope. This heats the individual wires and strands of the rope which in turn heat the plastic foaming composition causing it to soften and become plastic and causing the foaming agent to expand and foam the plastic as seen in FIG. 8. FIG. 9a shows a section of rope 71 which has already been foamed in a previous step. The interstices between the strands 75 and between the individual wires 73 within the strands are completely impregnated with a tough, flexible adherent plastic foam which completely excludes corrosive agents from the interior of the rope.

and strands and provides a cushion between the strands.

If as frequently occurs the original plastic coating on the individual wires has been damaged during stranding into the wire rope no damage is done to the finished wire rope since any nicks or scratches on the plastic coating on the wires are completely healed over by the foaming step and the individual strands and the interstices between the strands are completely filled with adherent plastic foam.

FIG. 10 shows an apparatus adapted for the continuous impregnation of a finished helical wire rope with a foam composition as shown in FIG. 9a. A catapulter type mold apparatus 85 has a series of molded rubber molds 87 attached to two endless chains 89 passing around sprocket wheels 91. The inner surface of each mold has a spiral configuration to match the surface configuration of the rope. Sprocket wheels 91 may be power driven to effect or assist the passage of the rope 93 or the apparatus may be driven by the passage of the rope. As the molds 87 are carried around sprockets 91 they close together over rope 93 as seen in cross-section in FIG. 11, and the spiral configurations on their inner surface close over the strands of the rope. The spiral on each mold 87 matches the spiral on adjacent molds so that the spiral configuration continues from one mold to the next to form a continuous spiral on the walls of the mold opening matching the lay of the strands of the wire rope. The spiral configuration on the mold surfaces is arranged to repeat as consecutive full lay lengths of strand pass through the mold apparatus 85. Different sets of molds are attached to endless chains 89 for different sized ropes and different rope lay lengths.

The molded rubber molds 87 do not normally need to have auxiliary cooling as the molds are continuously exposed to the cooling effects of the atmosphere for at least half of each revolution of the catapulter apparatus and each provides a fairly effective heat sink to remove heat from the surface of the wire rope, particularly if carbon is included in the rubber to increase the thermal conductivity.

A split induction coil 95 is mounted within the catapulter mold apparatus 85 surrounding the inner group of molds as they pass along the midline of the apparatus clamped together over the wire rope 93. As the rope 93 passes through split induction coil 95 its individual wires and strands are heated to melt and foam the surrounding plastic composition to impregnate the strands with plastic foam and fill the interstices in the interior of the rope between the strands with plastic foam. The rubber dielectric material of the molds 87 is not heated by the induction coil 95 so that the outer surface of the rope is kept relatively cool by the mold sections preventing excessive surface foaming and forming a thin layer 97 of fairly dense solidified plastic near the surface of the strands as best shown in the finished rope in FIG. 9a and in FIG. 9b, an enlarged section of FIG. 9a, to prevent the foam in the interior of the rope from escaping from the strands and rope prior to complete solidification.

Other dielectric materials besides rubber can be used for the molds so long as they can be effectively conformed about the strand or rope and are sufficiently heat conductive. The strand could also, of course, be

heated by other means than induction heating such as by steam jackets or the like and in such case the molds would not be required to be made from a dielectric material. Induction heating, however, is the most convenient and effective method of heating as it heats the strand or rope cross-section uniformly while allowing the surface to be kept cool to suppress excessive foaming in this area. Thus a solidified film or layer 97 of dense plastic forms near the surface of the strand or rope to contain the internal foam and provide a wear resistant plastic surface. If induction heating is not used the strand and rope must be heated from the exterior necessitating a more tightly conforming mold on the surface during heating to control the foaming, and a more sophisticated cooling section or cycle to confine the foam until an outer solidified layer of plastic 97 is formed.

The individual wires can be coated with the foaming composition in other ways than shown in FIGS. 1 and 2. In addition to coating from a bath of a suspension or emulsion of the plastic in a solvent, the wires can be coated by spraying, roller coating and other means. One particularly effective method of coating the wires with a thermoplastic coating composition is by extrusion. The wire is passed through a pressure extrusion head which maintains the plastic under pressure as long as it is melted so that the foaming agent cannot expand. After extrusion of the coating on the wire the wire will usually be wound on a reel for use on a stranding machine. Thereafter the wires are stranded into wire strand and ultimately in most cases into wire rope and the plastic foamed either in the strand or the rope.

I claim:

- 35 1. A wire strand having a tough, flexible plastic foam composition completely filling the interstices between the wires of the strand and adherent to the wires to seal the strand against corrosive agents and moisture and provide cushioning between the wires without significant reduction in wire density.
- 40 2. A wire rope having a tough, flexible plastic foam composition completely filling the interstices between the wires of the strands and between the strands in the interior of the rope and adherent to the said wires and strands to seal the strand against corrosive agents and moisture and provide cushioning between the wires and the strands without significant reduction in wire density.
- 45 3. A plastic impregnated wire strand comprising:
  - a. a plurality of metallic wires stranded together,
  - b. a tough, flexible plastic foam composition filling the interstices between the wires of the strand and adherent to the wires,
  - c. a solidified layer of dense plastic of substantially the same composition as the plastic foam of (b) adjacent to the surface of the strand and encapsulating the plastic foam within the strand.
- 50 4. A plastic impregnated wire strand according to claim 3 wherein the wire density of the strand is not substantially less than the wire density of a similar unimpregnated wire strand having identical metallic components and lay arrangement.
- 55 5. A wire strand according to claim 3 wherein the strand is a parallel wire strand.
- 60 6. A wire strand according to claim 3 wherein the strand is a helical wire strand.

65

7. A wire strand according to claim 4 wherein the strand is a parallel wire strand.

8. A wire strand according to claim 4 wherein the strand is a helical wire strand.

9. A plastic impregnated wire rope comprising:

- a. a plurality of wire strands stranded together,
- b. a tough, flexible plastic foam composition substantially completely filling the interstices between the wires of the component strands and between the strands in the interior of the rope and adherent to the wires,
- c. a solidified layer of dense plastic of substantially the same composition as the plastic foam of (b) adjacent to the surface of the rope and encapsulating the foam within the rope.

10. A plastic impregnated wire rope according to claim 9 wherein the wire density of the component strands of the rope is not substantially less than the wire density of a similar unimpregnated wire strand having identical metallic components and lay arrangement.

11. A method of fabricating a plastic foam impregnated wire strand comprising:

- a. coating the individual wires of the strand with a foamable plastic composition,
- b. forming the wires into a strand, and
- c. foaming the plastic foam composition within a closely confining mold surrounding the strand by

the application of heat to the strand.

12. A method of fabricating a plastic foam impregnated wire strand according to claim 11 wherein said strand is heated by induction-heating means while confined within a mold composed of a dielectric material.

13. A method of fabricating a plastic foam impregnated wire strand according to claim 12 wherein said mold is cooled by a cooling agent.

14. A method of fabricating a plastic foam impregnated wire rope comprising:

- a. coating individual wires with a foamable plastic composition,
- b. forming the coated wires into a strand,
- c. forming the strands into a rope, and
- d. foaming the plastic foam composition within a closely confining mold surrounding the wire rope by the application of heat to the wire rope.

15. A method of fabricating a plastic foam impregnated wire rope according to claim 14 wherein said rope is heated by induction-heating means while confined within a mold composed of dielectric material.

16. A method of fabricating a plastic foam impregnated wire rope according to claim 15 wherein said mold is cooled by a cooling agent.

\* \* \* \* \*

30

35

40

45

50

55

60

65